

# United States Patent Office

3,017,334

Patented Jan. 16, 1962

1

3,017,334

**ZINC BRUSH PLATING SOLUTION**  
Griffin L. Jones, 2166 Waverly, San Antonio 1, Tex.  
No Drawing. Filed Sept. 6, 1960, Ser. No. 54,327  
1 Claim. (Cl. 204—55)  
(Granted under Title 35, U.S. Code (1952), sec. 266)

The invention described herein may be manufactured and used by or for the Government for governmental purposes without payment to me of any royalty thereon.

This invention pertains to a new and an improved zinc brush plating solution for covering metal surfaces with a protective layer of zinc.

As a background for insuring a sufficient understanding of the present invention as claimed, the brush plating of protective coats on metal surfaces may be exemplified by U.S. Letters Patent No. 2,061,592, issued to Felix R. Rapids on Composition for and Method of Metal Electroplating.

In the past, baths for plating zinc on metals commonly have contained cyanide that is objectionably toxic. Issued patents wherein cyanide plating baths are described are No. 2,543,545, issued to Charles L. Faust et al. on February 27, 1951, and No. 2,451,426, issued to Robert R. Bair et al. on October 12, 1948. Other zinc plating baths are disclosed in Patents No. 2,799,635, issued to Allan E. Chester et al. on July 16, 1957, and No. 2,651,610, issued to Allan E. Chester on September 8, 1953.

A general statement of the nature and of the substance of this invention as claimed is a plating bath for use in the application of a protective layer of zinc on a metal surface and the composition of the plating bath.

An object of this invention is to provide a new and an improved zinc plating bath composition for use in the application of a protective coating of zinc on a metal surface.

The zinc plating bath that is contemplated hereby, is made up under ordinary laboratory conditions of temperature, pressure and humidity by adding together in a glass beaker or other suitable container the following materials:

|                   |                                 |
|-------------------|---------------------------------|
| Zinc sulfate      | 150 grams per liter of solution |
| Zinc acetate      | 200 grams per liter of solution |
| Ammonium chloride | 30 grams per liter of solution  |
| Boric acid        | 30 grams per liter of solution  |
| Mannitol          | 50 grams per liter of solution  |

2

Hydrochloric acid (concentrated) 100 cc. per liter of solution and enough distilled water to make 1 liter of solution; or

5 Zinc sulfate From 10 to 20 ounces per gallon of solution  
Zinc acetate 28 ounces per gallon of solution  
Ammonium chloride 5 ounces per gallon of solution  
Boric acid 5 ounces per gallon of solution  
Mannitol 7 ounces per gallon of solution

10 Hydrochloric acid (concentrated) 380 cc. per liter of solution and enough distilled water to make 1 gallon of solution.

The combined reagents are heated gently to get them all into solution. Any residue or cloudiness that remains in the solution cooled to room temperature of about 20 to 25° C. and at a pressure of about 1 atmosphere, is removed by filtration.

The mannitol in the above plating bath is a hexahydric alcohol of the composition  $C_6H_{14}O_6$  with the structural formula  $(CH_2OH)_2(CHOH)_4$  and is used as an addition in electroplating to transform weak tribasic boric acid into its stronger monobasic form. Several stereo-isomers of the compound are known.

15 It is to be understood that the zinc brush plating solution that is disclosed herein is submitted as an illustrative embodiment of the present invention and that limited modifications may be made therein without departing from the scope of this invention.

20 I claim:  
A zinc brush plating solution of the composition:

Zinc sulfate 150 grams per liter of solution  
Zinc acetate 200 grams per liter of solution  
Ammonium chloride 30 grams per liter of solution  
25 Boric acid 30 grams per liter of solution  
Mannitol 50 grams per liter of solution  
Concentrated hydro-

chloric acid 100 cc. per liter of solution  
and enough distilled water to make one liter of solution.

40 References Cited in the file of this patent

UNITED STATES PATENTS

694,658 Meurant Mar. 4, 1902  
45 2,029,387 Pine Feb. 4, 1936

UNITED STATES PATENT OFFICE  
CERTIFICATE OF CORRECTION

Patent No. 3,017,334

January 16, 1962

Griffin L. Jones

It is hereby certified that error appears in the above numbered patent requiring correction and that the said Letters Patent should read as corrected below.

Column 2, line 5, for "10" read -- 19 --; same column 2, lines 6 and 33, for "Zince", each occurrence, read -- Zinc --.

Signed and sealed this 19th day of June 1962.

(SEAL)

Attest:

ERNEST W. SWIDER  
Attesting Officer

DAVID L. LADD  
Commissioner of Patents